

Oct. 22, 1963

R. A. KOZLIK ET AL  
UNFIRED PRESSURE VESSEL  
Filed July 31, 1961

3,107,997



INVENTORS  
ROLAND A. KOZLIK  
CHARLES J. NEMK  
BY

*G. Dr. Weller*  
ATTORNEY

1

3,107,997

## UNFIRED PRESSURE VESSEL

Roland A. Kozlik, Livingston, and Charles J. Novak, Scotch Plains, N.J., assignors to The International Nickel Company, Inc., New York, N.Y., a corporation of Delaware

Filed July 31, 1961, Ser. No. 128,218  
11 Claims. (Cl. 75—124)

The present invention relates to austenitic stainless steels and, more particularly, to nickel-containing stainless steels and the manufacture of structures therefrom.

It is well known that extra-low carbon grades of nickel-containing stainless steels have many metallurgically attractive advantages which have led to their adoption in many areas of manufacturing. However, for the production of unfired pressure vessels for use up to and above 800° F., these grades of stainless steels have substantially limited commercial utilization since the engineering boiler codes have imposed extremely severe stress penalties attendant their use and, as a matter of fact, do not authorize the use of certain grades of stainless steel for unfired pressure vessels operating at temperatures in excess of 800° F. These officially imposed stress penalties are based in part upon a recognition that steels within the normally accepted composition limits for low and extra-low carbon stainless steels have widely varying high temperature stress characteristics which could not heretofore with certainty be predicted. In view of this fact, the extra-low carbon grades of nickel-containing stainless steels are not now commercially accepted for use in unfired pressure vessels operating at temperatures of the order of 500° F. to 800° F. or higher, regardless of whatever other attractive advantages may be afforded by the alloys. Although many attempts were made to provide extra-low carbon stainless steels which can be employed in unfired pressure vessels used at high temperatures, none, as far as we are aware, was entirely successful when carried into practice commercially on an industrial scale.

It has now been discovered that by maintaining specified and coordinated ranges of elements inherently co-present with nickel, chromium and iron in commercially produced stainless steels in a further coordinated relationship with specified amounts of alloying ingredients, stainless steels can be provided which are particularly suited for the manufacture of pressure vessels employable at elevated temperatures.

It is an object of the present invention to provide a novel stainless steel pressure vessel for use at elevated temperatures of the order of 800° F. and higher.

Another object of the invention is to provide a novel and improved method for the production of stainless steel structures such as pressure vessels utilizable at temperatures of the order of 800° F. and higher.

The invention also contemplates providing a unique stainless steel particularly adapted to be employed in the construction of pressure vessels utilizable at temperatures of the order of 800° F. and higher.

Other objects and advantages will become apparent from the following description taken in conjunction with the accompanying drawing which is a graphical plot of the effective factor of an alloy as hereinafter defined versus the boron content thereof.

Generally speaking, the present invention contemplates the manufacture of articles, structures and the like, such as unfired pressure vessels operable at temperatures of the order of about 800° F. to about 1200° F., from wrought alloys consisting essentially in weight percent of about 8% to about 14% nickel, about 15% to about 21% chromium, about 0.0015% to about 0.03% boron, about 0.008% to about 0.08% nitrogen, up to about 2% man-

2

ganese, up to about 0.15% carbon, up to about 0.2% aluminum, up to about 0.5% copper, up to about 1% silicon, with the balance being essentially iron together with correlated and controlled amounts of one or more of the elements columbium, titanium, vanadium and molybdenum, in addition to closely restricted amounts of elements unavoidably present as impurities in commercially manufactured stainless steels. The alloys from which the articles of the present invention are formed by working techniques including rolling, forging, extrusion and the like are adjusted while molten prior to casting to contain up to about 0.25% columbium, up to about 0.2% vanadium, up to about 0.25% titanium and up to about 1% molybdenum. The wrought alloys operable in accordance with the present invention are stably austenitic and can contain silicon in amounts up to 1%, for example, about 0.4% to about 0.9%, but the silicon content is advantageously so controlled that when the alloy contains less than about 0.02% carbon, 10% nickel and 0.03% nitrogen, the sum of the percentages of silicon and chromium does not exceed about 19.8%.

In the manufacture of the articles of the present invention and, in particular, when manufacturing said articles by hot working an air melted alloy which contains at least about 0.02% nitrogen, less than about 0.01% titanium and advantageously less than about 0.03% carbon, care must be taken to avoid excessive amounts of contaminating impurities during all stages of manufacture including melting, casting, working, welding, machining and the like. Low melting metals such as lead should be held to an absolute minimum in the alloy composition. Thus, lead which can be picked up during melting, casting, etc., should be present in the alloy of the finished article in amounts no greater than, for example, about 0.01%. Tin and zinc should likewise be maintained at as low a level as is commercially practical. Phosphorus and sulfur advantageously are maintained at a maximum of about 0.02% each. Zirconium in the alloy of the finished article should be no greater than about 0.02% and, advantageously, is less than 0.01%.

When making articles in accordance with the present invention, a molten bath of alloy is produced and adjusted in composition so that the alloy as cast therefrom and as subsequently worked and formed, contains interrelated amounts of nitrogen and one or more of the elements columbium, vanadium, titanium and molybdenum which in turn are related in a particular manner to the boron content. The effective amount of columbium and/or vanadium and/or titanium and/or molybdenum and nitrogen in the alloy articles of the present invention termed, for convenience, the effective factor (E.F.) of the alloy, are defined by the appropriate algebraic expression set forth in Table I in which percent (when used in conjunction with a chemical symbol of an element) indicates the numerical value of the percentage by weight of said element. As indicated in Table I, the effective factor of the alloy is determined with reference to the particular contents of titanium and nitrogen in the alloy.

Table I

| 4% N to percent Ti | Effective factor                                                     |
|--------------------|----------------------------------------------------------------------|
| <−0.01.....        | 7.8 [percent Ti to 4% N minus 0.01] plus K* <sup>1</sup> .           |
| −0.01 to 0.....    | K* <sup>1</sup> .                                                    |
| >0 to 0.12.....    | 4.9 [4% N to percent Ti] plus K* <sup>1</sup> .                      |
| >0.12 to 0.22..... | 1.5 [4% N to percent Ti minus 0.12] plus K* <sup>1</sup> plus 0.588. |
| >0.22.....         | 0.4 [4% N to percent Ti minus 0.22] plus K* <sup>1</sup> plus 0.738. |

<sup>1</sup> K\* equals 6% Cr plus 1.9% V plus 0.9 [percent Mo minus 0.2] minus 2 [percent Cu minus 0.28]. When the quantity [percent Mo minus 0.2] or the quantity [percent Cu minus 0.28] employed in the definitions set forth in Table I is equal to a negative number, it is to be disregarded and treated as equal to zero.

In order to provide useful structures adapted to be employed in the temperature range of 800° F. to about 1200° F. in accordance with the concepts of the present invention, it is necessary to correlate the E.F. of the alloy comprising said structure with the boron content thereof. As mentioned heretofore, this correlation is essentially inverse and is more particularly exemplified as set forth in Table II.

Table II

| Percent boron <sup>1</sup> | Minimum E.F., percent |
|----------------------------|-----------------------|
| 0.0015                     | 1.33                  |
| 0.005                      | 1.28                  |
| 0.008                      | 1.07                  |
| 0.010                      | 1.02                  |
| 0.015                      | 0.94                  |
| 0.020                      | 0.86                  |
| 0.025                      | 0.78                  |
| 0.030                      | 0.70                  |

<sup>1</sup> Determined by spectrographic analyses which analyses closely approximate boron percentages added to alloy following final deoxidation.

This relationship between the minimum effective factor of the alloy and the percentage of boron is also exemplified in the drawing. Referring now thereto, it is to be observed that articles in accordance with the present invention are made from alloys which are adjusted in composition so as to be represented by a point lying to the right of the curve when the boron content is plotted against the effective factor of the alloy.

In carrying the invention into practice, it is advantageous to adjust the composition of the molten bath so that the cast alloy which is wrought into the novel articles of the present invention contains amounts of alloying ingredients as set forth in Table III correlated as set forth hereinbefore.

Table III

| Element | Range, Percent       |                      |                      |                      |                      |
|---------|----------------------|----------------------|----------------------|----------------------|----------------------|
|         | Alloy A              | Alloy B              | Alloy C              | Alloy D              | Alloy E              |
| Ni      | 9-12                 | 9-12                 | 9-12                 | 9-12                 | 9-12                 |
| Cr      | 16-19                | 16-19                | 16-19                | 16-19                | 16-19                |
| Mn      | 1-2                  | 1-2                  | 1-2                  | 1-2                  | 1-2                  |
| Si      | 0.3-0.9              | 0.3-0.9              | 0.3-0.9              | 0.3-0.9              | 0.3-0.9              |
| B       | 0.0015-0.008         | 0.010-0.025          | 0.0015-0.008         | 0.003-0.025          | 0.002-0.025          |
| Cb      | 0.1-0.15             | 0.15 max.            | 0.1-0.15             | 0.1-0.15             | 0.10-0.15            |
| C       | 0.015-0.035          | 0.015-0.035          | 0.015-0.035          | 0.015-0.035          | 0.08 max.            |
| N       | 0.03-0.04            | 0.03-0.04            | 0.01-0.04            | 0.01-0.04            | 0.03-0.06            |
| Ti      | 0.01 max.            | 0.01 max.            | 0.04 max.            | 0.1 max.             | 0.1 max.             |
| V       | 0.15 max.            | 0.15 max.            | 0.1-0.15             | 0.10-0.15            | 0.15 max.            |
| Al      | 0.1 max.             | 0.1 max.             | 0.1 max.             | 0.1                  | 0.1 max.             |
| Cu      | 0.3 max.             | 0.3 max.             | 0.3 max.             | 0.5 max.             | 0.3 max.             |
| Mo      | 0.7 max.             | 0.7 max.             | 0.7 max.             | 0.7 max.             | 0.7 max.             |
| Fe      | Bal. E. <sup>1</sup> | Bal. E. <sup>1</sup> | Bal. E. <sup>1</sup> | Bal. E. <sup>1</sup> | Bal. E. <sup>1</sup> |

<sup>1</sup> Balance essentially.

In correlating the alloying ingredients to adjust the composition of the alloy in accordance with the concepts of the present specification and claims, it is to be noted that for any given alloy range the effective factor of the alloy is defined with respect to the ranges of nitrogen and titanium. For example, with respect to Alloy A as set forth in Table III, since 4 times (×) the percentage of nitrogen (percentage N) minus (—) the percentage of titanium (percentage Ti), i.e., the nitrogen-titanium factor (N-T-F), can be a maximum of 0.16 and a minimum of 0.11 the effective factor of this alloy is defined when the nitrogen-titanium factor is from 0.11 up to 0.12 by the expression

$$6 \times \% \text{Cb} + 1.9 \times \% \text{V} + 0.9 [\% \text{Mo} - 0.2] - 2 [\% \text{Cu} - 0.28] + 4.9 [4 \times \% \text{N} - \% \text{Ti}]$$

and when the nitrogen-titanium factor is in excess of 0.12 the E.F. of the alloy is defined by the expression

$$6 \times \% \text{Cb} + 1.9 \times \% \text{V} + 0.9 [\% \text{Mo} - 0.2] - 2 [\% \text{Cu} - 0.28] + 1.5 [4 \times \% \text{N} - \% \text{Ti} - 0.12] + 0.588$$

70  
75

After the molten bath of the alloy is so adjusted, the alloy is cast and wrought to form heat-resistant articles. The articles thus made in accordance with the present invention exhibit excellent high temperature stability when subjected to temperatures of the order of 800° F. to 1200° F. by virtue of the fact that they are comprised of a non age-hardenable alloy possessing a coordinated chemical composition specifically designed to minimize the formation of deleterious microstructures when subjected for extended periods of time to stress at elevated temperatures.

To illustrate more fully the advantages of the present invention, alloys illustrative of alloys which can be employed in the novel process and articles of the present invention are set forth in Table IV.

Table IV

| Element | Percent by weight    |                      |                      |                      |                      |
|---------|----------------------|----------------------|----------------------|----------------------|----------------------|
|         | Alloy No. 1          | Alloy No. 2          | Alloy No. 3          | Alloy No. 4          | Alloy No. 5          |
| Ni      | 10.95                | 11.01                | 9.4                  | 10.3                 | 11.14                |
| Cr      | 18.68                | 18.5                 | 18.7                 | 16.4                 | 18.5                 |
| Mn      | 1.11                 | 1.2                  | 1.19                 | 1.31                 | 1.17                 |
| Si      | 0.48                 | 0.5                  | 0.56                 | 0.67                 | 0.3                  |
| C       | 0.017                | 0.032                | 0.02                 | 0.015                | 0.05                 |
| N       | 0.031                | 0.031                | 0.022                | 0.029                | 0.054                |
| V       | 0.04                 | 0.082                | 0.12                 | 0.12                 | 0.016                |
| Cb      | 0.12                 | 0.03                 | 0.12                 | 0.14                 | 0.14                 |
| Ti      | <0.01                | <0.01                | 0.014                | 0.03                 | <0.01                |
| Al      | 0.098                | 0.027                | <0.01                | <0.01                | 0.012                |
| B       | 0.0015               | 0.017                | 0.0024               | 0.0053               | 0.019                |
| Cu      | -----                | 0.09                 | 0.30                 | 0.34                 | -----                |
| Mo      | -----                | <0.01                | 0.25                 | 0.64                 | <0.01                |
| Fe      | <sup>1</sup> Bal. E. | <sup>1</sup> Bal. E. | <sup>1</sup> Bal. E. | <sup>1</sup> Bal. E. | <sup>1</sup> Bal. E. |

<sup>1</sup> Balance essentially.

When formed into wrought articles, the alloys set forth in Table IV are ductile, weldable and exceptionally resistant to the deleterious effects of stress at elevated

temperatures of the order of 1200° F. The data in Table V shows the 100-hour rupture stress at 1200° F. in pounds per square inch (p.s.i.) of articles made from the alloys set forth in Table IV.

Table V

| Alloy No. | 100-hour rupture stress at 1200° F. (p.s.i.) | Alloy No. | 100-hour rupture stress at 1200° F. (p.s.i.) |
|-----------|----------------------------------------------|-----------|----------------------------------------------|
|           |                                              | 65        | 65                                           |
| 1         | 33,200                                       | 4         | 37,500                                       |
| 2         | 35,000                                       | 5         | 38,500                                       |
| 3         | 36,250                                       |           |                                              |

The data set forth in Table V is to be compared to data with regard to alloys which are similar in chemical composition but which are outside the scope of the present invention. The 100-hour rupture stress of such similar alloys outside the scope of the present invention can be as low as 18,000 p.s.i. or even 15,000 p.s.i. In addition, al-

## 5

loys outside the scope of the present invention can form deleterious microstructural constituents during processing or service in articles exposed to elevated temperatures. Thus, if the articles contain too much chromium, molybdenum and/or silicon and/or too little nickel, carbon and/or nitrogen, deleterious amounts of ferrite can form in the substantially completely austenitic matrix of the alloy article. Excessive amounts of columbium, molybdenum and titanium can induce the formation of deleterious carbides. Excessive amounts of vanadium tend to reduce ductility and increase the tendency of the alloy articles to be notch sensitive. When nitrogen is present in the alloy in amounts in excess of about 0.01%, amounts of titanium in excess of about 0.01% are to be avoided in order to minimize and/or eliminate the formation of deleterious amounts of titanium nitrides and/or carbonitrides. To minimize the formation of deleterious amounts of carbides, the carbon content of the alloy articles of the present invention must not exceed 0.15%, should not exceed about 0.10% or 0.08% and, advantageously, is less than 0.03%. Excessive amounts of aluminum over 0.2% can weaken the alloy articles of the present invention. Excessive amounts of boron can induce undue difficulties in welding said articles but advantageously at least about 0.002% boron is present in the alloys. When producing the alloy articles in accordance with the present invention, small amounts of cobalt can be introduced along with nickel and small amounts of tantalum can be introduced along with columbium. Such small incidental amounts of cobalt and tantalum are not deleterious to the characteristics of the alloy articles of the present invention.

Alloy articles made in accordance with the present invention and adapted to be employed at temperatures of the order of 800° F. and higher, exhibit 100-hour rupture stresses at least in excess of 30,000 p.s.i. at 1200° F. Such alloy articles include hydrogenation equipment, high temperature oil and steam piping, superheater elements, furnace parts such as retorts, muffles, radiant tubes, mesh belts, chain link belts, etc., heat exchangers, etc.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. An unfired pressure vessel for use at temperatures of about 800° F. to about 1200° F. made of a stable, non-age hardenable austenitic alloy consisting essentially of about 8% to about 14% nickel, about 15% to about 21% chromium, about 0.0015% to about 0.03% boron, about 0.008% to about 0.08% nitrogen, up to about 2% manganese, up to about 0.15% carbon, up to about 0.2% aluminum, up to about 0.25% titanium, up to about 0.5% copper, up to about 1% silicon, up to about 0.25% columbium, up to about 0.2% vanadium, up to about 1% molybdenum with the balance being essentially iron, the elements in said alloy being so correlated that when the effective factor of said alloy is plotted against the boron content thereof, the alloy is representable by a point lying to the right of the curve in the accompanying drawing.

2. An unfired pressure vessel in accordance with claim 1 made of an alloy containing up to about 0.08% carbon.

3. An unfired pressure vessel in accordance with claim 1 made of an alloy containing less than about 0.01% titanium.

4. An unfired pressure vessel in accordance with claim

## 6

1 made of an alloy containing up to about 0.035% carbon.

5. An unfired pressure vessel in accordance with claim 4 made of an alloy containing less than about 0.01% titanium.

6. An unfired pressure vessel in accordance with claim 4 made of an alloy containing at least about 0.002% boron.

7. An unfired pressure vessel for use at temperatures of about 800° F. to about 1200° F. made of a stable, non-age hardenable austenitic alloy consisting essentially of about 9% to about 12% nickel, about 16% to about 19% chromium, about 0.0015% to about 0.003% boron, about 0.03% to about 0.04% nitrogen, about 1% to about 2% manganese, about 0.015% to about 0.035% carbon, up to about 0.1% aluminum, up to about 0.01% titanium, up to about 0.3% copper, about 0.3% to about 0.9% silicon, about 0.1% to about 0.15% columbium, up to about 0.15% vanadium, up to about 0.7% molybdenum with the balance being essentially iron, the elements in said alloy being so correlated that when the effective factor of said alloy is plotted against the boron content thereof, the alloy will be represented by a point lying to the right of the curve in the accompanying drawing.

8. An unfired pressure vessel for use at temperatures of about 800° F. to about 1200° F. made of a stable, non-age hardenable austenitic alloy consisting essentially of about 9% to 12% nickel, about 16% to 19% chromium, about 0.01% to about 0.25% boron, about 0.03% to about 0.04% nitrogen, about 1% to about 2% manganese, about 0.015% to about 0.035% carbon, up to about 0.1% aluminum, up to about 0.01% titanium, up to about 0.3% copper, about 0.3% to about 0.9% silicon, up to about 0.15% columbium, up to about 0.15% vanadium, up to about 0.7% molybdenum with the balance being essentially iron, the elements in said alloy being so correlated that when the effective factor of said alloy is plotted against the boron content thereof, the alloy will be represented by a point lying to the right of the curve in the accompanying drawing.

9. An unfired pressure vessel for use at temperatures of about 800° F. to about 1200° F. made of a stable non-age hardenable austenitic alloy consisting essentially of about 9% to about 12% nickel, about 16% to about 19% chromium, about 0.0015% to about 0.003% boron, about 0.01% to about 0.04% nitrogen, about 1% to about 2% manganese, about 0.015% to about 0.035% carbon, up to about 0.1% aluminum, up to about 0.04% titanium, up to about 0.3% copper, about 0.3% to about 0.9% silicon, about 0.1% to about 0.15% columbium, up to about 0.15% vanadium, up to about 0.7% molybdenum with the balance being essentially iron, the elements in said alloy being so correlated that when the effective factor of said alloy is plotted against the boron content thereof, the alloy will be represented by a point lying to the right of the curve in the accompanying drawing.

10. An unfired pressure vessel for use at temperatures of about 800° F. to about 1200° F. made of a stable, non-age hardenable austenitic alloy consisting essentially of about 9% to about 12% nickel, about 16% to about 19% chromium, about 0.003% to about 0.025% boron, about 0.01% to about 0.04% nitrogen, about 1% to about 2% manganese, about 0.015% to about 0.035% carbon, up to about 0.1% aluminum, up to about 0.1% titanium, up to about 0.5% copper, about 0.3% to about 0.9% silicon, about 0.1% to about 0.15% columbium, about 0.10% to about 0.15% vanadium, up to about 0.7% molybdenum with the balance being essentially iron, the elements in said alloy being so correlated that when the effective factor of said alloy is plotted against the boron content thereof, the alloy will be represented by a point lying to the right of the curve in the accompanying drawing.

11. An unfired pressure vessel for use at temperatures of about 800° F. to about 1200° F. made of a stable, non-age hardenable austenitic alloy consisting essentially of about 9% to about 12% nickel, about 16% to about 19% chromium, about 0.002% to about 0.025% boron, about 0.03% to about 0.06% nitrogen, about 1% to about 2% manganese, up to about 0.08% carbon, up to about 0.1% aluminum, up to about 0.1% titanium, up to about 0.3% copper, about 0.3% to about 0.9% silicon, about 0.1% to about 0.15% columbium, up to about 0.15% vanadium, up to about 0.7% molybdenum with

the balance being essentially iron, the elements in said alloy being so correlated that when the effective factor of said alloy is plotted against the boron content thereof, the alloy will be represented by a point lying to the right of the curve in the accompanying drawing.

References Cited in the file of this patent

UNITED STATES PATENTS

|           |              |       |               |
|-----------|--------------|-------|---------------|
| 2,562,854 | Binder       | ----- | July 31, 1951 |
| 2,602,028 | Urban et al. | ----- | July 1, 1952  |
| 2,750,283 | Loveless     | ----- | June 12, 1956 |

UNITED STATES PATENT OFFICE  
CERTIFICATE OF CORRECTION

Patent No. 3,107,997

October 22, 1963

Roland A. Kozlik et al.

It is hereby certified that error appears in the above numbered patent requiring correction and that the said Letters Patent should read as corrected below.

Column 1, line 66, for "nad" read -- and --; column 2, lines 60 to 68, Table I, should appear as shown below instead of as in the patent:

| 4% N -- % Ti  | Effective Factor                        |
|---------------|-----------------------------------------|
| <-0.01        | : 7.8 [% Ti - 4% N - 0.01] + K*         |
| -0.01 to 0    | : K*                                    |
| >0 to 0.12    | : 4.9 [4% N - % Ti] + K*                |
| >0.12 to 0.22 | : 1.5 [4% N - % Ti - 0.12] + K* + 0.588 |
| >0.22         | : 0.4 [4% N - % Ti - 0.22] + K* + 0.738 |

column 6, line 30, for "0.25%" read -- 0.025% --.

Signed and sealed this 12th day of May 1964.

(SEAL)  
Attest:

ERNEST W. SWIDER  
Attesting Officer

EDWARD J. BRENNER  
Commissioner of Patents